

No. 789,523.

PATENTED MAY 9, 1906.

A. G. BETTS.

PROCESS OF ELECTROLYTICALLY REFINING COPPER-NICKEL ALLOYS.

APPLICATION FILED APR. 11, 1904.

FIG. 1



FIG. 5



FIG. 2



FIG. 3



FIG. 4



FIG. 6



FIG. 7



WITNESSES

Edward F. Kern.  
William Valentine

INVENTOR

Auson G. Betts

## UNITED STATES PATENT OFFICE.

ANSON GARDNER BETTS, OF TROY, NEW YORK.

## PROCESS OF ELECTROLYTICALLY REFINING COPPER-NICKEL ALLOYS.

SPECIFICATION forming part of Letters Patent No. 789,523, dated May 9, 1905.

Application filed April 11, 1904. Serial No. 202,603.

*To all whom it may concern:*

Be it known that I, ANSON GARDNER BETTS, a citizen of the United States, residing at Troy, in the county of Rensselaer and State of New York, have invented new and useful Improvements in Processes of Electrolytically Refining Copper-Nickel Alloys, of which the following is a specification accompanied by drawings.

10 Figure 1 of the drawings is a vertical section of the apparatus for electrolytically dissolving the copper-nickel alloy and depositing copper. Figs. 2 and 5 are vertical sections of different forms of apparatus for electrolytically depositing nickel. Figs. 3 and 6 are vertical sections showing apparatus arranged for electrolytically reducing lead sulfate contained in spongy lead to metallic lead. Figs. 4 and 7 are vertical sections of apparatus in 15 which copper-nickel alloy is dissolved in sulfuric acid.

This invention relates to a process of making pure nickel and pure copper from alloys containing copper and nickel.

20 In electrolytically refining copper alloys containing considerable quantities of nickel by the usual electrolytic copper - refining process, using an acid copper-sulfate solution as electrolyte, the solution becomes enriched 25 in nickel by the accumulation of nickel sulfate. To electrolytically deposit the nickel and recover the combined sulfuric acid in useful form has been a difficult and expensive matter; and the object of my invention is to 30 reduce this difficulty and cost.

In practicing my invention I first electrolytically dissolve the copper-nickel alloy and simultaneously deposit pure copper in and from an acid solution of sulfate of copper. 35 The nickel dissolved from the anodes remains in the solution as sulfate, while a chemically-equivalent amount of copper is deposited on the cathodes. The solution accordingly increases in concentration with respect to nickel 40 sulfate and decreases in respect to copper sulfate. Accordingly I occasionally withdraw solution of nickel and copper sulfate from the refining-tanks, replacing it with fresh solution of copper sulfate containing perhaps some 45 nickel sulfate to keep plenty of copper in the

copper-depositing solution. The nickel-sulfate solution I free from copper by well-known electrolytic or chemical methods and prepare a pure nickel-sulfate solution therefrom by crystallization of nickel sulfate or by freeing the 55 solution from impurities by chemical methods. The pure nickel-sulfate solution is electrolyzed with an anode of spongy lead of the same character as is used for the negative electrodes of lead storage batteries, whereby nickel is deposited on the cathode and the lead partly converted into lead sulfate. I then electrolyze a solution of sulfuric acid with the spongy-lead electrode as cathode and prefer to use a lead-peroxid electrode, partly reduced to lead 60 sulfate as anode, whereby the solution becomes enriched in sulfuric acid, the lead sulfate of the spongy-lead electrode being reconverted into spongy lead for further use in depositing nickel from the solution of its sulfate and the lead sulfate of the lead-peroxid electrode being converted into lead peroxid, as in charging a lead storage battery. If the lead-peroxid electrode is used, after it is thoroughly peroxidized I bring it into a solution 65 containing sulfuric acid in which is also suspended an electrode of copper or nickel-copper alloy, or fragments of such metal may be supported therein on a conductor. On closing the circuit electric energy is generated, 70 with the conversion of a part of the lead peroxid into lead sulfate and solution of the copper-nickel or copper anode. The electric energy produced may be most easily utilized by placing the cell in the refinery-circuit, when 75 it operates to raise the voltage of the current passing through instead of depressing the voltage, as in the case of most electrolytic tanks. The copper-sulfate or nickel-copper-sulfate solution produced goes to the electrolytic copper-depositing and copper-nickel-dissolving tank. My process is therefore regenerative 80 as regards the sulfuric acid used and partly as regards the electric energy used. I may, however, use a plain lead anode or one of 85 other insoluble material in this operation.

An alternative method in reducing the lead sulfate of the spongy-lead electrode consists in electrolyzing with a plain lead anode and neutralizing the sulfuric acid produced by 90 95 100

dissolving therein copper oxids or metallic copper with the help of oxidation by means of air, which operations can be easily carried out by well-known methods. The copper-sulfate solution produced is added to the copper-depositing electrolyte.

Referring to the accompanying drawings, Fig. 1 shows in vertical section a tank 1, lined with lead 2, containing a solution 3 of copper and nickel sulfates and an anode 4 of copper-nickel alloy being refined. When an electric current is passed, copper and nickel dissolve from the anode and copper 6 deposits on copper cathodes 5.

Fig. 2 shows in vertical section a tank 7, lined with lead 8. On the bottom of the tank is a layer of spongy lead 9. The tank contains a solution of nickel sulfate 10, in which is suspended a cathode 11, of suitable material, with its electrodeposit of nickel 12. When an electric current is passed, nickel deposits on the cathode and the spongy lead is partly converted into lead sulfate.

Fig. 3 shows in vertical section the same tank 7 and spongy lead 9, with a solution of sulfuric acid 13, in which is suspended a lead electrode 14, containing in recesses in its body active material of lead, lead peroxid, and lead sulfate 15. When an electric current is passed, the lead sulfate in the spongy lead is converted into metallic lead and the lead sulfate in the active material 15 is converted into lead peroxid and the concentration of sulfuric acid in the electrolyte increases exactly as in the case of charging a lead storage battery when charging.

Fig. 4 shows in vertical section a tank 16, lined with lead 17, on the bottom of which is a layer of copper-nickel-anode scrap 18 or other copper-nickel fragments or metallic copper. The lead electrode 14 with its active material in a peroxidized condition is suspended in the contained solution 19 of sulfuric acid. When an electric current is allowed to pass, the lead peroxid of the electrode 14 is partly converted into lead sulfate and metal is dissolved from 18, with the production of electric energy.

Fig. 5 shows in vertical section a form of apparatus which can be used in place of that shown in Fig. 2. The tank 20, lined with lead 21, contains a solution 22 of nickel sulfate. An electrode 23, of lead, containing in recesses in its body spongy lead 24, is suspended in the solution. Cathodes 25, of suitable material, with their electrodeposits of nickel 26, are also suspended in the solution. The electrochemical solution is the same as was described under the description of Fig. 2.

Fig. 6 shows a view in vertical section of a form of apparatus which can be used in place of that shown in Fig. 3. The tank 27 contains the lead electrode 23, (shown in Fig. 5,) with the active material in the condition of containing lead sulfate in a solution 29 of sul-

furic acid. Lead electrodes 30, containing in recesses in their bodies plugs 31, of active material of lead, lead sulfate, and lead peroxid in the reduced condition, are suspended in the solution. The electrochemical operation is the same as was described under the description of Fig. 3.

Fig. 7 shows in vertical section a form of apparatus which can be used in place of that shown in Fig. 4. The tank 32, lined with lead 33, contains a solution of sulfuric acid 34, with the electrodes 30, (shown in Fig. 6,) with the active material 31 in a peroxidized condition suspended therein and an anode 35, of copper alloy. The electrochemical operation is the same as that described under the description of Fig. 4.

What I claim as new, and desire to secure by Letters Patent, is—

1. The process of electrodepositing nickel from solutions of nickel sulfate, which consists in electrolyzing the solutions with an anode of spongy lead, and with a suitable cathode.

2. The process in refining copper-nickel alloys, which consists in dissolving the alloy as anode in a solution containing copper salts, for the electrodeposition of metallic copper and production of a solution of nickel salt, preparing a nickel-sulfate solution therefrom, electrolyzing the nickel-sulfate solution with a suitable cathode and with a spongy-lead anode for the electrodeposition of metallic nickel, and production of lead sulfate, and reducing the lead sulfate formed to metallic lead by electrolysis as a cathode in a solution containing the sulfuric-acid radical.

3. The process of electrolytically depositing metallic nickel from solutions of nickel sulfate, which consists in electrolyzing the solution with a suitable cathode and with an anode of spongy lead, and subsequently reducing the lead sulfate produced by electrolysis as a cathode in a solution of sulfuric acid.

4. The process of refining copper-nickel alloys which consists in electrolyzing a solution of copper and nickel sulfates, with the alloy as anode, preparing nickel-sulfate solution from the nickel-and-copper solution, electrolyzing the nickel-sulfate solution with a spongy-lead anode, with the deposition of nickel on a suitable cathode, electrolytically reducing to spongy lead the lead sulfate formed, for the production of sulfuric-acid solution, converting the sulfuric acid obtained partly into copper sulfate, and returning the copper sulfate to the copper-depositing bath.

5. The process of refining copper-nickel alloys which consists in electrolyzing a solution of copper and nickel sulfates, with the alloy as anode, preparing nickel-sulfate solution from the nickel-and-copper solution, electrolyzing the nickel-sulfate solution with a spongy-lead anode, with the deposition of nickel on a suitable cathode, electrolytically

reducing to spongy lead the lead sulfate formed, for the production of sulfuric-acid solution, converting the sulfuric acid obtained partly into copper sulfate by electrolysis of said sulfuric acid with an anode containing copper, and a cathode of lead peroxid, and returning the copper sulfate formed to the copper-depositing bath.

In testimony whereof I have signed my name to this specification in the presence of two subscribing witnesses.

ANSON GARDNER BETTS.

Witnesses:

EDWARD F. KERN,  
WILLIAM VALENTINE.